

## UNITED STATES PATENT OFFICE

2,339,740

PHTHALOCYANINE AZO DYES ON  
CELLULOSIC FIBERS

Harold Blackshaw and Norman Hulton Haddock,  
Blackley, Manchester, England, assignors to  
Imperial Chemical Industries Limited, a cor-  
poration of Great Britain

No Drawing. Application May 22, 1942, Serial No.  
444,107. In Great Britain September 25, 1939

8 Claims. (Cl. 8—46)

The present invention relates to the coloring of cellulosic fiber, this application being a continuation-in-part from our copending application Serial No. 355,692, filed September 6, 1940. More particularly this application relates to dyeing or printing of cellulosic fiber by impregnating the same with a diazotized poly-amino-phthalocyanine compound, and subsequently submitting the impregnated fiber to an after-treatment as hereinafter described, to develop a water-insoluble azo dye on the fiber.

This invention is based on the discovery that diazotized di-, tri- and tetra-amino-phthalocyanines have affinity for cellulosic fibers, which they dye in the same way as, for example, diazo dyestuffs derived from benzidine, and that by treating the cellulosic fibers with the said diazotized poly-amino-phthalocyanines, in the manners described below, brown and violet to green and grey shades of good fastness properties are obtained thereon.

When we speak of diazotized poly-amino-phthalocyanines, we are referring to compounds obtainable by treating di-, tri- or tetra-amino-phthalocyanines, for instance tetra-amino-copper-phthalocyanine, tetra-amino-cobalt-phthalocyanine, tetra-amino-metal-free-phthalocyanine, or their homologs, analogs and nuclear substitution derivatives, such as chloro, nitro alkyl and alkoxy, with various quantities of nitrous acid, to diazotize at least some of the amino groups. The preferred procedure is to use sufficient nitrous acid to diazotize theoretically all the amino groups present in the molecule. But even here there is no certainty as to the number of diazonium groups in the final compound, because the resulting compound is generally not stable and may undergo partial decomposition before it has a chance to be applied to the fiber.

The aftertreatment is carried out by treating the cellulosic fiber, which has been impregnated with the diazotized poly-amino-phthalocyanine, with azo-dye coupling components which are free of sulfo, carboxy or similar water-solubilizing groups. Principal consideration among these deserve the azoic, or so-called "ice-color," coupling components. These are typified by  $\beta$ -naphthol, 2-hydroxy-3-naphthoic anilide, bis-acetoacet-o-toluidide, 1-phenyl-3-methyl-5-pyrazolone, resorcinol,  $\alpha$ -naphthol, 2:3-hydroxy-naphthoic-o-toluidide, 2:3-hydroxynaphthoic-p-anisidine and the p-chloranilide of 2-hydroxycarbazole-3-carboxylic acid.

As equivalents coming within the scope of this

invention may be mentioned other coupling components free of water-solubilizing groups, such as phenol, p-cresol, aceto-acetic ester, and aceto-acet-p-phenetidide, as well as coupling components which per se are soluble but can be converted into water insoluble compounds on the fiber by lactamization. See, for instance, U. S. Patents Nos. 2,012,994; 2,012,991 and 2,098,276.

The said coupling component may be applied to the fiber which has been dyed or printed with the phthalocyanine diazo compound, in any convenient manner. The coupling components are then applied from solutions prepared in the usual manner, for instance by the aid of alkali, as is customary in carrying out azoic couplings.

In reaction with the coupling components the diazotized aminophthalocyanines are presumed to yield primary azo dyestuffs, in which it is understood that the diazonium nitrogen atoms remain intact.

Accordingly, the present invention relates to a process for dyeing or printing cellulosic fiber, which comprises impregnating the fiber with a solution or printing paste containing a diazotized poly-amino compound of the phthalocyanine series, and subsequently treating the impregnated fiber in such a manner as to develop a water-insoluble azo dye on the fiber. In this way, according to this invention, there are obtained on cellulosic fibers brown or violet to green and grey shades of good fastness properties, including fastness to washing.

For dyeing, the cellulosic fiber, e. g. cotton or regenerated cellulose, is conveniently treated with the diazotized poly-amino-phthalocyanine by immersing it at 0°-30° C. in an aqueous solution of the latter. The diazotized tetra-amino-phthalocyanines usable as starting materials are described in copending application of Haddock, Serial No. 335,871 (Patent No. 2,280,072, issued April 21, 1942), and may be obtained by the process set out therein. The corresponding compounds of lesser diazo content may be prepared by reducing and diazotizing in similar manner the dinitro and trinitro-phthalocyanines described in British Patent No. 541,146 (p. 2, lines 104-111; p. 4, lines 68-78).

Taking the tetra-amino-phthalocyanine of copper as typical, the same may be diazotized ready for use, or there may be employed acidified solutions of the metallic double salts of the diazotized tetra-amino-phthalocyanine, or the corresponding alkali-metal isodiazotates. Metallic tetra-amino-phthalocyanines other than those of copper may be used for preparing diazo com-

pounds suitable for use in the process of the invention; for example, those of magnesium, cobalt, nickel, lead or aluminium, which are conveniently prepared by heating the appropriate metal or metal salt with a nitrophthalonitrile and reducing the resulting tetra-nitrophthalocyanine. Metal-free tetra-amino-phthalocyanines can also be used.

The invention is illustrated but not limited by the following examples in which the parts are 10 by weight.

*Example 1*

To a stirred suspension of 2 parts of copper tetra-(4)-amino-phthalocyanine in 40 parts of water mixed with 50 parts of 33% aqueous hydrochloric acid, at 5° C., there is rapidly added a solution of 1 part of sodium nitrite dissolved in 20 parts of water. The dark-green solution so obtained is filtered and diluted to 1400 parts with equal quantities of ice and water.

Into 350 parts of the diazonium solution thus obtained, 10 parts of cotton yarn are immersed for 1 hour at 10° C., with occasional turning. The yarn is then immersed for 10 minutes in a solution of 0.5 part of  $\beta$ -naphthol dissolved in 250 parts of 0.1% sodium hydroxide solution at 30° C. The material is then taken out, rinsed in cold water and dried. A violet shade of excellent fastness to washing is produced.

Instead of  $\beta$ -naphthol there may be employed 2-hydroxy-3-naphthoic anilide. By this means a similar violet shade of similar fastness properties is obtained.

Other violet shades are obtained by employing 2:3-hydroxynaphthoic o-toluidide or 2:3-hydroxynaphthoic p-anisidine in place of  $\beta$ -naphthol. By using instead of  $\beta$ -naphthol the p-chloranilide of 2-hydroxycarbazole-3-carboxylic acid a grey shade is produced.

Similar shades are also obtained by using tetra-diazotized cobalt or nickel tetra-(4)-amino-phthalocyanine in place of tetradiazotized copper tetra-(4)-amino-phthalocyanine.

*Example 2*

10 parts of cotton yarn are impregnated with diazo compound as in Example 1 and are then introduced into a solution of 0.5 part of bis-acetoacet-o-toluidide in 250 parts of 0.1% sodium hydroxide solution. The cotton is dyed in a yellowish-green shade of very good fastness to washing and of good fastness to light.

If resorcinol is used in place of bis-acetoacet-o-toluidide an olive-green shade is produced, having good fastness to washing. If 1-phenyl-3-methyl-5-pyrazolone is used in place of bis-acetoacet-o-toluidide, a yellowish-green shade of good fastness to washing is produced.

*Example 3*

Copper-tetra-(4)-amino-phthalocyanine is azotized as in Example 1 and filtered. Cotton cloth is padded with the undiluted filtrate in such a way as to leave an amount of the diazo solution equal in weight to the weight of the dry cloth in the fiber. Coupling of the diazo on the fiber to phenol is carried out by stirring the impregnated fabric in a solution containing 1 gram of phenol per liter of water and sufficient sodium hydroxide to maintain brilliant yellow 70 alkalinity, at about 5° C. The cloth is rinsed in water and dried. By this treatment, there results a dyeing green in shade with excellent washing fastness and good light fastness.

If, in the place of the phenol above, aceto-

acetic ester is used, a brighter green dyeing with similar washing and light fastness results. Olive green dyeings are obtained if aceto-acet-p-phenetidine or phenyl-methyl-pyrazolone is employed. With  $\beta$ -hydroxy-naphthoic anilide, a dull violet dyeing is obtained. In all cases, dyeings with very good washing fastness and good light fastness are obtained.

*Example 4*

Copper tetra-(4)-amino phthalocyanine is azotized as in Example 1, and filtered. The acidity of the filtrate is then adjusted by the addition of sodium acetate until it reaches a pH-value of approximately 3. This solution is then thickened to a printing paste by the addition of a thickener, as for example gum tragacanth. Cotton cloth is printed with this paste. Coupling with beta-hydroxy-naphthoic-anilide is effected by turning the printed fabric in a solution containing 2 grams of this coupling component per liter of water and sufficient sodium hydroxide to maintain Clayton Yellow alkalinity, the temperature being maintained at approximately 5° C. The cloth is then rinsed in cold water, soaped, rinsed again, and dried. There results a print of dull violet shade, which displays excellent washing fastness and good light fastness.

Cotton cloth is printed with a printing paste consisting of the potassium isodiazotate derived from copper phthalocyanine tetra-(4)-diazonium chloride (obtained as described below), bis-acetoacet-o-toluidide, neutral starch-tragacanth thickening, Turkey red oil and water. After steaming for ten minutes, soaping, rinsing and drying, a bright green print is obtained which has very good wash fastness and good light fastness.

The potassium tetra-(4)-iso-diazotate of copper phthalocyanine hereinabove mentioned may be made as follows:

30 parts of finely divided copper tetra-(4)-amino-phthalocyanine in the form of an aqueous paste are mixed with 350 parts of water and 150 parts of concentrated aqueous hydrochloric acid (sp. gr. 1.16). To the mixture at 5° C. is added a solution of 15 parts of sodium nitrite in 50 parts of water. The temperature is maintained throughout at 5° C. or below. The dark green diazo solution is now added to a stirred mixture at -10° C. of 1200 parts of potassium hydroxide and 800 parts of water. The green solution so obtained is added rapidly to a mixture of 1600 parts of potassium hydroxide and 400 parts of water previously heated to 120°. The temperature is maintained at not less than 120° C. during the addition. The mixture is cooled to 100° C. and the tetra-isodiazotate, in suspension, is filtered off through asbestos paper. It is pressed under vacuum till dry. The product is a dark green powder soluble in cold water to give a bluish green solution.

In most of the examples above, the diazo solution of tetra-amino copper phthalocyanine has been indicated as freshly prepared and used immediately, in view of its tendency to decompose on standing. If desired, instead of the free diazonium compound, acid solutions of its double salts with inorganic compounds, for instance zinc chloride, or its compounds with aromatic sulfonic acids, for instance, 1,5-naphthylene-disulfonic acid, may be used. (See U. S. Patent No. 2,280,072). We have found, incidentally, that a considerable degree of stabilization may be achieved by adding surface-active quaternary

ammonium compounds, such as long-chain-alkyl-pyridinium-halides. Thus we have found that the addition to the dye bath of 0.25% of cetyl-pyridinium bromide in the presence of free hydrochloric acid would stabilize the tetradiazonium derivative of tetra-(4)-amino-copper-phthalocyanine to such an extent that after 2 hours at 17° C., the amount of decomposition found was slight.

In lieu of the tetradiazon compound obtained from copper-tetra-(4)-amino-phthalocyanine employed in the above examples, there may be used with equal success the tetra-diazo-compound from copper-tetra-(3)-amino-phthalocyanine, the tridiazon compound obtained from copper-tri-(4)- or tri-(3)-amino-phthalocyanine, the bis-diazo compound from copper-diamino-phthalocyanine, also the corresponding diazonium compounds derived from cobalt and nickel tetra-amino and tri-amino-phthalocyanines, and the diazonium compounds derived from tetra-amino and tri-amino metal-free phthalocyanines.

The dyeings obtained on cellulosic material according to this invention are all characterized by good fastness to washing, soap boiling, open soda boiling, and light.

It will be understood that the detailed practice of our invention is susceptible to wide variation and modification within the skill of those engaged in this art.

We claim:

1. A process for coloring cellulosic fiber, which comprises impregnating the same with a polydiazonium compound obtained by diazotizing a polyamine of the phthalocyanine series, and then subjecting the impregnated fiber to treatment with a coupling component adapted to develop a water-insoluble azo dye on the fiber.

2. A process for coloring cellulosic fiber, which comprises impregnating the same with a polydiazonium compound obtained by diazotizing a polyamine of the phthalocyanine series, and then subjecting the impregnated fiber to treatment

with an azo coupling component devoid of sulfo and carboxy groups.

3. A process for dyeing cellulosic fiber, which comprises impregnating the same with a solution of a polydiazonium compound obtained by diazotizing a tetra-amino-compound of the phthalocyanine series, and then treating the impregnated fiber with a solution of an azoic coupling component to produce a water-insoluble dyestuff on the fiber.

4. A process for dyeing cellulosic fiber, which comprises impregnating the same with an aqueous solution of a polydiazonium compound obtained by diazotizing a tetra-amino-copper-phthalocyanine, and then treating the impregnated fiber with a solution of an arylide of aceto-acetic acid.

5. A process for dyeing cellulosic fiber which comprises impregnating the same with tetradiazotized copper-tetra-(4)-amino-phthalocyanine, and then treating the impregnated fiber with a solution of an azoic coupling component selected from the group consisting of  $\alpha$  and  $\beta$ -naphthol, the monohydroxy and dihydroxy-benzenes, the 1-aryl-3-methyl-5-pyrazolones, the esters and arylides of aceto-acetic acid, and the arylides of 2,3-hydroxy-naphthoic acid and of 2-hydroxy-carbazole-3-carboxylic acid.

6. Cellulosic textile material colored with azo coloring matters developed on the fiber by a process as defined in claim 1.

7. Cellulosic textile material dyed with azo coloring matters by a process as defined in claim 5.

8. A process for dyeing cellulosic fiber, which comprises impregnating the fiber with an aqueous solution of the poly-diazonium compound obtained by diazotizing tetra-amino-copper phthalocyanine, and then treating the impregnated fiber with an azoic coupling component to produce a water-insoluble poly-azo dyestuff on the fiber.

HAROLD BLACKSHAW.  
NORMAN HULTON HADDOCK.